

## [54] METHOD OF PRODUCING BLISTER COPPER

3,890,139 6/1975 Suzuki et al. .... 75/74  
 4,006,010 2/1977 Rajcevic et al. .... 75/74  
 4,032,327 6/1977 Donaldson et al. .... 75/72

[75] Inventors: Stig A. Petersson; Bengt S. Eriksson, both of Skelleftehamn, Sweden

Primary Examiner—M. J. Andrews  
 Attorney, Agent, or Firm—Stevens, Davis, Miller & Mosher

[73] Assignee: Boliden Aktiebolag, Stockholm, Sweden

## [57] ABSTRACT

[21] Appl. No.: 774,454

A method of producing blister copper comprising smelting sulphidic copper raw material in a rotary furnace with an inclined rotation axis, in presence of oxygen and slag formers charged simultaneously with the copper raw material. The method comprises discontinuing the oxygen charge when at least 75% of the copper raw material has been charged and treating the obtained matte and slag with a reduction agent and then transferring the matte and the slag together to a holding furnace in which the matte and the slag are separated and transferring the matte in the holding furnace to a converter where it is converted to blister copper.

[22] Filed: Mar. 4, 1977

10 Claims, 1 Drawing Figure

## [30] Foreign Application Priority Data

Mar. 12, 1976 [SE] Sweden 76032382

[51] Int. Cl.<sup>2</sup> C22B 15/06

[52] U.S. Cl. 75/73

[58] Field of Search 75/72, 74, 76, 24, 73, 75/75

## [56] References Cited

## U.S. PATENT DOCUMENTS

3,666,440 5/1972 Kono et al. .... 75/76  
 3,682,623 8/1972 Dierckx et al. .... 75/76





## METHOD OF PRODUCING BLISTER COPPER

The present invention relates to a method of producing blister copper from sulphidic copper material, the sulphidic copper material being smelted down discontinuously in a furnace to form a matte having a high copper content and a slag having a relatively low copper content, whereafter the molten material, comprising slag and matte, is transferred to a settling furnace in which the slag is treated to reduce the copper content thereof, whereafter the slag and the copper matte are continuously tapped-off together. The copper matte is then after separation from the slag converted to blister copper in a conventional manner.

Principally, blister copper is produced from sulphidic copper material by methods comprising three stages these being a first stage in which the material is roasted, a second stage in which the roasted product is smelted and a third stage in which the copper-sulphide smelt is converted to blister copper by blowing or injecting into the smelt an oxygen-containing gas, normally air, the iron oxides being slagged at the same time, by adding an acid flux, such as silica, e.g. sand, to the process. A characteristic feature of such conventional copper processes is that they are all effected in stages. By roasting the sulphidic copper material, i.e. heating the material by supplying oxygen to combust sulphur present in the material, there is obtained a partial combustion of sulphide sulphur (i.e. the sulphur contained in the sulphide), this combustion process being controlled to ensure that the roasted product contains sufficient sulphur to form a matte having the desired copper content during the subsequent smelting process. Normally, the matte contains 30-40% copper and 22-26% sulphur. The chemical composition of the matte will, of course, vary in dependence upon the nature of the ingoing raw material and the extent to which roasting is effected. The aforementioned copper and sulphur ranges, however, are representative of matte produced from those copper raw-materials most commonly used.

In addition to obtaining matte when smelting sulphidic copper material, there is also obtained an iron-containing slag which is imparted a suitable composition by adding sand ( $SiO_2$ ) and, in certain cases, minor quantities of limestone, thereby to impart a low viscosity to the slag. The slag, which normally contains approximately 0.4-0.8% copper, is tapped-off and discarded. In certain cases the slag may also contain significant quantities of zinc and other valuable metals, which metals can be recovered in slag-fuming processes.

In conventional, batchwise, smelting processes, the copper content of the matte is regulated to 30-40%, since a higher copper content would result in a higher copper content of the slag, which would lead to unacceptable copper losses.

Over the years, a number of mutually different smelting furnaces have been constructed. The design of these furnaces is normally such as to require copper raw-materials together with a slag-former to be continuously charged to the furnace and there smelted. The slag and copper matte can be tapped-off continuously or discontinuously.

A usual type of smelting furnace in this context is the reverberatory furnace comprising, in principle, a long and narrow furnace space having a rectangular bottom, the furnace space being heated by means of oil or gas burners. Air, or air enriched with oxygen-gas is charged

to the furnace for the oil or gas combustion. Reverberatory furnaces are now being replaced to an ever increasing extent by other types of smelting furnaces, partly for reasons of an economic nature and partly for reasons of an environmental nature, since it has been found extremely difficult to recover effectively the sulphur dioxide-containing gases generated during the smelting process. Reverberatory furnaces namely generate large volumes of gas, which means that large and expensive gas-purification systems must be provided. One way of avoiding this problem is to smelt the material by means of electrical energy. An electric smelting furnace suitably comprises a long and narrow surface space having a rectangular bottom in which electrodes are arranged, normally electrodes of the Söderberg type, which are intended to be immersed in the material to be smelted. The energy required to carry out the smelting process is obtained by resistance heating techniques. The electric furnaces represent a considerable step forward in the art and improve the possibilities of purifying and recovering generated gases, owing to the fact that the furnace can operate under a specific, controllable pressure lower than the ambient pressure, so as to avoid unacceptable leakage of deleterious substances from the furnaces, which substances may be harmful to the environment, and because less gas need be generated than that generated in the reverberatory furnace, thereby enabling smaller gas-purification systems to be used. In order for electric smelting furnaces to be economic, however, access must be had to inexpensive electric power.

The aforementioned smelting processes normally provide a copper matte containing 30-40% copper, and an outgoing slag containing between 0.4 and 0.8% copper, this slag being discarded. It is desirable, however, to produce in the smelting process a matte with the highest possible copper content, for example a copper content of 60-77%, preferably 65-75% Cu. The production of a smelt of such high copper content has not been possible in hitherto known copper-smelting processes, however, because too much copper is lost to the slag. When converting matte having a low copper content in discontinuous Pierce-Smith converters or in previously known processing apparatus according to known processes, a very large quantity of slag containing 4-8% copper is obtained, which slag must be returned to the smelting process or cooled down, crushed and subjected to flotation processes in order to recover the copper content of the slag. This incurs significant expense. A further disadvantage encountered in known copper conversion processes, is that part of the iron contained by the slag is oxidized to form magnetite, which owing to its high melting point will remain substantially in solid form and settle in the melting unit to form deposits therein when the slag is returned.

It has been found in practice that if the copper content of the matte is raised during smelting process to more than 40%, the copper content of the slag will be so high as to render the copper losses unacceptable.

A further disadvantage with the aforementioned smelting processes is that the copper material must normally be sintered or roasted before it is charged to the furnace. Consequently, in latter years smelting apparatus have been developed in which it is possible to smelt copper concentrates directly and in which the heat used to effect the smelting process is provided by heat generated upon the combustion of sulphur contained in the concentrates, i.e., by so-called autogenous

smelting. One such furnace is the so-called flash-smelting furnace which, in principle, comprises a vertically arranged reaction shaft, a horizontally arranged settling-furnace portion for the molten material and a waste-gas section. Pre-heated air and dried concentrates are charged to the top of the reaction shaft. An exothermic reaction takes place in the tower between the oxygen in the air and the sulphur in the copper concentrate, the concentrate particles reaching smelting temperature and then falling down into the settling-furnace portion, in which they form a molten bath comprising copper matte and slag. Normally, the slag is tapped continuously from such furnaces whilst the copper matte is tapped off discontinuously. The copper content of the matte can be regulated by controlling the supply of oxygen to the process, the copper content normally lying at about 60% and the slag containing 0.8-2.0% copper. Since slag containing such large quantities of copper must be refined, for economic reasons, the slag is treated in a separate furnace in which the copper content can be reduced to 0.4-0.8%.

In addition to furnaces of the aforementioned type (Outokumpu) other furnaces of the INCO type can be mentioned, these furnaces operating in accordance with the same principles, the main difference being that furnaces of the Outokumpu type use pre-heated air when smelting the concentrate in the shaft, while the furnaces of the INCO type use oxygen-gas enriched air in the absence of a flash shaft.

In addition to the high copper content primarily obtained in the slag, a further disadvantage encountered with flash furnaces is that they are unsuitable for melting scrap and/or oxidic material.

Copper matte produced in accordance with previously known processes is subsequently transferred to a copper converter in which residual sulphur is oxidized, by blowing air or oxygen-containing gas into the converter in a conventional manner, to form blister copper and sulphur dioxide.

During the past years a multiplicity of continuous copper-producing processes have been developed, in which the steps of smelting the raw-materials, slagging the iron contained in said materials and converting the resultant matte to blister copper are all carried out in a single furnace or in a plurality of mutually combined units. Normally, blister copper and slag are tapped continuously from the furnace. A continuous copper-producing process was described as early as 1898 by Garrison in U.S. Pat. No. Spec. 596,992, in which the steps of smelting copper-containing materials and converting the same to copper, and separating the copper from the slag were all effected in one and the same furnace.

Thus, the above U.S. Patent Specification describes the continuous smelting of sulphides in a furnace heated by fuel-burners and having a long, narrow bottom which slopes but very slightly. The matte obtained thus flows continuously to one or more separate but interconnected converters arranged in series at one end of the furnace. The matte is blown continuously to form metal which is tapped-off. The slag obtained, which is rich in copper, flows continuously back in counter-current to the matte, through the furnace to a separate but communicating slag-separating zone at the other end of the furnace and is subjected there to heat and to a reduction process with charcoal; copper which is reduced out is taken up into the matte, which is separated and permitted to flow back to the furnace, whereafter the thus purified slag is tapped-off.

In 1954 there was described in U.S. Pat. No. Spec. 2,668,107 (INCO) a process comprising the autogenous smelting of copper-sulphide and nickel-sulphide concentrates by injecting dry sulphides and a flux by means of oxygen gas, optionally also air, into a closed furnace. Matte or white metal, and slag forms continuously and is collected on the bottom of the furnace, whereafter the matte or white metal is tapped from one end of the furnace and the slag from the other end. According to this patent, the metal-rich slag is purified in counterflow to the matte. The slag is allowed to pass a threshold or barrier in the hearth so as to separate the slag from the matte and the white metal and other metals formed, whereafter the slag is treated with a shower of molten matte droplets having a low copper content but rich in iron sulphide, whereafter the slag thus treated is tapped-off.

In the U.S. Pat. Nos. Spec. 3,004,846 and 3,030,201, 3,069,254, 3,468,629, 3,516,818, 3,615,361 and 3,615,362 (INCO) processes are described for converting copper-sulphide, nickel-sulphide and lead-sulphide materials into corresponding metals in rotary furnace units. Oxygen is injected into the furnace from above by means of downwardly projecting gas lances through which process gases of adjusted composition and of the desired temperature are directed onto and through the surface of the bath. These patents emphasize the importance of creating sufficient agitation in the furnace to ensure effective contact between the gases, the solid substances and the liquid material in the furnace, since in this way the removal of iron, sulphur and impurities, such as antimony and arsenic, is effectively promoted. When applying this principle, requiring a turbulent bath, the heat transfer and the rate at which chemical reactions take place are increased, owing to a significant decrease in the diffusion barriers between slag and sulphide phase. According to "Western Miner" November 1975, page 16-19, a copper-producing plant which is to operate in accordance with the aforementioned processes is planned in Canada.

In a publication by R. Schumann, Jr. in transactions AIME Vol. 188, 1950, page 8, "A Survey of The Thermodynamics of Copper Smelting" there is presented a thermodynamic analysis of conditions prevailing when smelting and converting mixtures of copper sulphides and iron sulphides to form copper metal and slag. This article reveals the importance of the activity of oxygen and sulphur, respectively, in the system, these activities being accorded the highest significance in respect of the thermodynamic relationships in copper smelting processes. The publication shows that in typical matte-slag systems, the equilibrium pressure can be varied over a wide range. This fact shows that it is difficult to optimize the copper content in the slag and matte in a manner such that the resultant copper content of the slag is sufficiently low and that the matte contains a sufficiently high content of copper. The partial pressure of oxygen at equilibrium in the system depends upon three stoichiometric factors determined by the material charged to the furnace, namely the matte concentration, the silica content of the slag and the ratio of oxygen to iron, the oxygen in the silica being discounted, and by the temperature.

During latter years many different processes have been proposed in attempts to solve problems encountered with the pyrometallurgical conversion of sulphide concentrates to metal in a continuous process, for example such processes as those described in the U.S. Pat.

Nos. Spec. 3,326,671 (Worcra), 3,542,352 (Noranda) and 3,687,656 (Metallgesellschaft).

In spite of all the efforts made, some serious problems still remain. The U.S. Pat. No. 3,326,671 describes a number of different furnace constructions for a process based on the concept of a furnace divided into three zones. When the process gases are injected from above through downwardly extending overhead tuyeres, or lances, complications and limitations are met in the operation of furnaces not provided with particular agitation means, mainly because the reactions are slower. If the speed at which the gas passes through the furnace is increased, so as to obtain more effective and rapid reactions, high dust losses are experienced, especially when the furnace is charged with dry concentrates which have not been sintered. (Compare U.S. Pat. No. 3,326,671, page 9, line 31). Furthermore, such a method renders it extremely difficult to produce a slag having the desired low copper content, since it is difficult in one and the same furnace unit to work simultaneously with a strongly oxidizing zone in close proximity with a strongly reducing zone, despite the fact that the slag in the reducing zone is not in direct contact with the matte or white metal (i.e., phases of higher copper content), the physical separation of the slag from matte or white metal being achieved by arrangements of structural members, such as threshold-type barriers.

The U.S. Pat. No. Spec. 3,542,352 describes a method in which, when smelting concentrate, there is applied a concurrent-process, while when separating copper from slag there is applied, subsequent to the slag having passed a threshold, barrier, a counter-flow process thereby to avoid contact between white metal and copper. In order to separate copper from the slag, a reducing gas is blown thereinto, the copper being reduced and running back to the main body of white metal and copper, said body being collected in front of the threshold in the furnace, from where it is tapped-off continuously. The slag is also tapped-off continuously. The disadvantage with the aforescribed process is that copper reduced out from the slag also dissolves impurities in the raw material, such as antimony and bismuth, which metals can cause serious disturbances in the subsequent electrolytic refinement of blister copper. The slag will also contain relatively high percentages of copper, which means that the slag must be treated subsequent to being tapped-off, either by flotation or by sulphide-treating processes effected in a separate furnace. The copper content of the slag reaches 9-12%, it being possible to reduce this content somewhat by reduction.

The U.S. Pat. No. Specification 3,687,656 (Metallgesellschaft) describes a semi-continuous method in which a series of complicated treatment stages are effected in a multi-chamber unit in which process gases are injected through downwardly directed gas lances.

The German Patent Application No. 2,322,516 (Mitsubishi) describes a method of continuously producing blister copper in three separate stages, these stages comprising a smelting furnace, a slag-purification furnace and a converter. In comparison with other continuous copper-producing processes, it is possible by the method of this German Application to control the slagging procedure more favourably. One disadvantage, however, is that the continuously operating smelting furnace can only be operated under oxidizing conditions, which results in a slag having a high copper content. According to the description of the German Ap-

plication, it is preferred to control the process in a manner such that only 60% of the copper contained in the sulphidic copper raw-material is recovered in the smelting process, since a higher content of copper in the matte would result in a very high copper content of the slag, the slag then being passed further to the slag purification furnace. When the smelting process is effected under oxidizing conditions, the slag will also contain high percentage of magnetite, which renders the slag highly viscous and difficult to handle.

In accordance with a recently published method, designated KIVCET, *Erzmetall* 28, pages 313-22 (1975) complex copper concentrates are charged to a furnace space in a vortex and smelted in said space, the smelt distributing itself between said furnace space and a further furnace space where reducing conditions are maintained whilst, for example, vaporizing zinc and other impurities. The smelting process in the first furnace space is effected under oxidizing conditions and flue gases are removed, by suction, to a purification plant. The atmosphere in the further furnace space is a strongly reducing atmosphere and hence the predominant portion of metallic impurities will be present in the matte phase, naturally with the exception of zinc and lead which depart in vapour form. Under special conditions it is also possible to vaporize tin and arsenic. The furnace, however, is not constructively suitable to control the conditions in the two furnace spaces and the possibility of obtaining desired conditions is apparently limited, particularly in the further furnace space.

Because of the oxidizing conditions maintained when smelting copper concentrates in accordance with the KIVCET method considerable quantities of magnetite are formed and hence the temperature must be maintained at a very high magnitude — 1600°-1800° C. — if a liquid slag is to be formed. This high temperature represents a serious disadvantage with respect to energy consumption and, in addition, the materials from which the furnace is constructed are seriously affected.

Despite the large number of processes known for producing copper, it has now surprisingly been found possible to devise a new process which offers a large number of advantages vis-à-vis the previously known processes.

The invention consists in a method of producing blister copper, wherein sulphidic copper raw material is smelted to form a matte and a slag in a rotary furnace arranged to rotate about an inclined axis at a rotary speed of from about 10 rpm to about 60 rpm in the presence of oxygen and slag formers and wherein the matte is converted to blister copper in the manner known per se, which method comprises the steps of heating the furnace to a temperature of at least 900° C. charging simultaneously the copper raw material, slag former and oxygen to the furnace to autogeneously smelt said raw material by means of heat obtained by burning sulphur contained in said raw material, so that a smelt comprising a matte having a desired copper content and a copper-containing slag is formed and maintained at a temperature of 1100°-1300° C.; treating the smelt obtained with at least one reductant selected from the group consisting of coke, coal, oil, natural gas, pyrite, chalcopyrite, pyrrhotite and additional amounts of said sulphidic copper raw material, so that the copper content in the slag is decreased; transferring the smelt batchwise to a holding furnace in which the matte and the slag are mutually separated; reducing the slag in the holding furnace during its passage therethrough by any

manner known per se to further decrease the copper content in the slag to a predetermined level; tapping off the matte separated in the holding furnace and transferring it to a converter; and finally tapping-off the slag thus reduced and separated.

The new process of the present invention comprises a surprising combination of known integers, which combination enables copper to be produced from widely differing raw materials, such as concentrates, copper-containing cinders and ashes and copper scrap. The method comprises charging sulphidic copper smelt material to a rotary furnace having an inclined axis of rotation, in which furnace the copper material is smelted whilst supplying oxygen and slag former to the furnace, although it must naturally be ensured that the sulphur content and oxygen content of the process gas supplied is sufficient to smelting the copper material in the manner desired. Thus, the oxygen content may vary between 25 and 100%, although a content of 30-50% is preferred. The resultant melt, comprising matte and slag, is then treated with a reductant. The whole melt, matte and slag, is then transferred to a holding furnace in which the slag and matte are mutually separated. The slag is further treated in the holding furnace to reduce the copper content of the slag, whereafter the slag is tapped-off, optionally for further treatment in a vaporizing furnace to recover zinc. The matte is transferred to a converter in which it is converted to blister copper in a manner known per se. Because of the reducing atmosphere, the magnetite content can be reduced to approximately 2%, which provides a slag of the required fluidity. Further, because the furnace rotates, it is possible to prevent the zinc present from vaporizing and accompanying the waste gas even though the magnetite content is so low. This is not at all possible in conventional processes. The oxygen supply is suitably discontinued when at least 75%, and preferably at least 85% of the copper raw material has been charged to the furnace. The remaining sulphidic copper raw material will then act as a reduction agent. Alternatively, all of the copper raw material may be charged to the furnace whilst supplying oxygen thereto, whereafter a reductant, such as coke, coal, oil, pyrite, chalcopyrite, or pyrrhotite, is charged to the furnace. During the smelting process, the temperature is maintained at between 1100° and 1300° C., preferably between 1150° and 1250° C. Prior to charging copper raw material to the furnace, the furnace is heated to a temperature of at least 900° C. by means of a burner.

The temperature of the holding furnace is maintained at 1150°-1250° C. with the aid of a burner or by means of resistance heating. The copper content of the slag is reduced in the holding furnace either by charging sulphidic concentrates, coke or coal to the furnace or by combusting a fuel therein with a reducing flame.

The novel process affords new and surprising advantages which, surprisingly, have not been previously realised by one skilled in this art, despite the fact that the problems associated with previous methods have been obvious.

The amount of energy consumed by the process is low, since the heat required for smelting the raw copper material is obtained by burning sulphur contained in the copper concentrate, i.e., so-called autogenous smelting. Smelting of the raw copper material can be effected with either roasted products obtained from conventional roaster furnaces or with copper concentrates, which may also be moist. With autogenous smelting

there is obtained a significant surplus of heat, especially when only oxygen gas is used, which surplus can be used to smelt copper scrap and/or be recovered in a waste heat boiler. The smelting process may suitably be remotely controlled from a control room, whereby no person need remain in the reactor hall during normal operation, thereby enabling difficultly solved internal environmental problems to be solved. Furthermore, the smelting unit itself may be so constructed as to be exchangeable with another, so that repair work, such as relining the furnace, may be done in places suitable therefor, thereby further improving internal environmental conditions. Since it is possible to construct the reactor hall in such a manner that it is in effect a closed locality, recovery and purification of process gases is greatly facilitated and the soiling of the ambient environment avoided thereby.

The smelting unit used in accordance with the new method is a rotary furnace which, in operation, rotates about an inclined axis. An example of such a furnace is the Kaldo converter which is also designated as top-blown rotary converter. Such a converter is arranged to rotate at such speeds that material is entrained from the bath by the wall and caused to fall down as droplets into the bath, thereby providing for particularly effective contact between the bath and the gas phase existing above the surface of the bath, thereby enabling very fast reactions to take place and to maintain equilibrium between the various parts of the bath. This speed can be calculated suitably as the peripheral speed of the inner wall of the cylindrical part of the furnace. The speed should be from 0.5 to 7 m/s, preferably from 2 to 5 m/s. This corresponds to a rotary speed of 10-60 r.p.m. depending upon the diameter of the furnace. A large furnace, in the order of magnitude of 5 m diameter, can reach a suitable peripheral speed already at a rotary speed of 10 r.p.m. while a very small furnace, less than one meter in diameter, should have a rotary speed of more than 40 r.p.m. The Kaldo converter is described exhaustively in, for example, Journal of Metals, April 1966, pages 485-490, and in Stahl und Eisen 86, (1966) pages 771-782.

As will be seen from this literature, a Kaldo converter comprises a cylindrical portion and a conical top section. The converter has a refractory lining and is provided with means by which it can be rotated at speeds of 10-60 r.p.m., these means having the form, for example, of a friction drive or a toothed-drive ring extending around the container and suitable drive means associated therewith. The whole of the rotatable converter together with the means for rotating the same can be tipped to the tap furnace. In other respects, the kaldo furnace is provided with conventional auxiliary equipments, such as supply devices, tuyeres or lances, gas purification equipment and control apparatus.

By charging raw material batchwise to a rotary furnace having an inclined axis of rotation, relatively rapid reactions are obtained and the process can be readily controlled by means of data processing apparatus, whereby the process can be quickly adjusted should the incoming raw material vary. Thus, the process affords important advantages, since a widely varying assortment of raw materials can be smelted and metalurgically treated with the desired result.

The holding furnace suitably has the form of a horizontally arranged furnace space, for example a long narrow furnace space having a rectangular bottom surface, in which material is charged at one end and slag

and matte are allowed to mutually separate during passage through the furnace. The slag is tapped-off at the other end of the furnace, slag being conveyed from the charging end of the holding furnace towards the slag-removal end. During its passage through the holding furnace, the slag is treated by adding sulphidic concentrates and/or a reductant such as coke or coal. Further, a reducing gas flame can be used for the reducing treatment process. As a result hereof, the copper content of the slag can be maintained at very low levels. This process also provides a sufficiently long treatment time, even if the process in the smelting stage is relatively rapid. Heat is applied to the holding furnace by using electric resistance heating techniques, such as Söderberg electrodes, or by means of a gas burner, which may be combined with the reducing treatment of the slag.

The matte, which contains very high percentages of copper, 65-75%, is then transferred to a converter of, for example, the conventional PS-type. The conversion of the matte may also be effected in a Kaldo converter, when this is found suitable, e.g. when it is desired to carry out simultaneously certain metallurgical treatment steps, such as steps in which the antimony content of matte is lowered. A conventional converter is preferred, however, when no special conditions prevail. Owing to the high copper content of the matte, small quantities of slag are formed during the conversion process, these affording important economic gains compared with previous methods since the converter slag is always very rich in copper, normally 6-8% copper.

A matte may contain between 18 and 77% copper and, in commercial copper processes, normally contains 30-60% copper. A matte having more than roughly 75% copper, may be termed a concentrated matte or white metal.

Thus, the process according to the present invention provides for extraordinary flexibility.

Since the smelting unit can be exchanged for a further smelting unit, stoppages in production caused by repair work are avoided and, except for the rare occasions when the holding furnace must be closed down for maintenance work, the system can be driven continuously. It is also possible, at times, to permit matte to be transferred from the rotary furnace directly to the converters, even though in such cases a somewhat poorer copper yield is obtained, since the slag will have a slightly higher copper content. Slag which has a slightly higher copper content can, if desired, be charged to the holding furnace when this furnace is again in operation. This is an extremely important advantage vis-à-vis the large number of copper processes based on integrated processes in one or more separate furnaces, in which when one process stage is closed down it is necessary to empty the plant and completely interrupt production. In order to safeguard against stoppages in production still further, the process apparatus may comprise a multiplicity of smelting units.

The process is illustrated schematically in the accompanying drawing, the single FIGURE of which shows a rotary furnace 1 having an inclined axis of rotation, the furnace being charged with copper raw material in the direction of arrow 2. When the furnace has been charged and the melt treated with a reductant, both the matte and the slag are transferred to a holding furnace 3 in the manner indicated by the arrow 4. The matte is transferred from the holding furnace 3 via means indicated by arrow 5 to a converter 6, while the slag is transferred to a zinc-vaporizing apparatus or a granulat-

ing apparatus via means indicated by arrow 7, and discarded. Copper is removed from the converter 6 by means indicated by arrow 8. Slag formed in the converter is returned to either the furnace 1 or the holding furnace 3 by means indicated by arrow 9.

The invention will now be illustrated with reference to a number of examples:

#### EXAMPLE 1

Fine-grain concentrate and slag former,  $\text{SiO}_2$ , such as sand, were charged continuously through a water-cooled lance to a Kaldo furnace having a capacity of approximately 5 tons whilst simultaneously charging oxygen, alternately oxygen-enriched air, through the lance in quantities as to obtain a matte smelt having the desired copper content. The oxygen content of the air charged to the furnace was adjusted so that the material charged to the furnace could be smelted autogeneously, this being achieved with an air charge containing 30-50%  $\text{O}_2$ . Thus, the oxygen content must be adjusted in accordance with the composition of the concentrate and to its moisture content and should in general be maintained within the ranges given for the majority of material. Subsequent to reaching the desired copper content of the matte, the air supply was discontinued whilst concentrates continued to be charged to the furnace until a further, approximately 10%, concentrates had been charged, whereby the copper content of the slag was reduced. During the reduction period, the furnace was kept heated by means of an oxygen gas-oil burner. Subsequent to the termination of the reduction period, the matte and the slag were tapped-off together, transferred and charged into one end of a rectangular holding furnace, in which sulphidic material was charged to one end thereof so as to reduce the percentage of copper in the slag to less than 0.4% in a manner known per se before tapping-off the slag. The matte was transferred to a conventional Pierce-Smith converter, in which the matte was blown with air to form copper.

| Result                   | % Cu |     | % Fe |    | % $\text{SiO}_2$ |      | % $\text{Fe}_3\text{O}_4$ |    |
|--------------------------|------|-----|------|----|------------------|------|---------------------------|----|
|                          | 1    | 2   | 1    | 2  | 1                | 2    | 1                         | 2  |
| Matte prior to reduction | 65   | 77  | 5.5  | 1  | —                | —    | —                         | —  |
| Matte after reduction    | 63   | 74  | 6.5  | 1  | —                | —    | —                         | —  |
| Slag prior to reduction  | 2.0  | 3.9 | 33   | 33 | 32               | 32.5 | 7                         | 14 |
| Slag after reduction     | 0.8  | 0.9 | 34   | 35 | 33               | 33   | 5                         | 7  |

As shown by the results of the two tests, subsequent to smelting raw copper material in the Kaldo furnace there was obtained a matte having a very high copper content whilst the copper content of the slag was very low, less than 1%. Slag having such low copper content cannot be obtained with previously known methods, despite the fact that the copper content of the matte has been much lower in said methods. The low copper content of the slag enables the holding furnace to operate continuously, since a further reduction of the copper content to less than 0.4% can be very rapidly achieved by treating the slag with sulphidic concentrates, coke or a reducing flame in the manner aforementioned.

Another example illustrates still more the high degree of flexibility of the copper process, since surprisingly it is possible to smelt and beneficiate antimony-rich copper raw material having >0.2% antimony without the antimony content of the copper produced subsequent to

conversion exceeding 400 g/t, which is necessary if it is to be possible to carry out a troublefree electrolysis in the final electrolytic-refining of the anode copper.

Another object of the invention is thus a method of smelting copper raw materials containing more than 0.2% antimony to a matte whilst simultaneously removing the antimony from said material, wherein the said copper raw materials are smelted in an inclined, rotary furnace together with an addition of iron containing slag, said iron containing slag being charged to the furnace in quantities such that the total amount of iron present in the furnace is at least 44 times of the antimony present in the furnace, whilst supplying heat from a burner, whereafter the resultant matte smelt, subsequent to tapping-off the slag, is converted in the same furnace by blowing with an oxygen containing gas through lances, to form white metal and a further slag, whereafter said further slag is removed.

The smelting is effected during a first phase by supplying heat from the burner with a reducing flame, preferably with an oxygen quantity charged corresponding at most 80% of the stoichiometrically required quantity, and during a second phase with an oxidizing flame, preferably with an oxygen quantity charged corresponding to at least 120% of the stoichiometrically required quantity. The temperature is increased to between 880°-980° C. by means of the reducing flame and to 1150°-1300° C. by means of the oxidizing flame. The furnace rotates with a peripheral speed at the cylindrical inner wall of the furnace of from 0.5 to 7 m/s, and preferably from 2 to 5 m/s.

Antimony will readily accompany the copper and the problem is serious especially if it is desired to produce a matte having a high copper content, 65-75% copper. In previously known processes there is also formed in such cases a minor quantity of metallic copper which immediately dissolves practically all the antimony present. The method comprises smelting the copper raw material in an inclined rotary furnace together with an addition of iron-containing slag in quantities such that the total quantity of iron in the furnace is at least 44 times the amount of antimony present in the furnace. Heat is supplied by means of a burner suitably fired with oil and oxygen gas, smelting suitably taking place in two different phases, in which the first phase is effected in a reducing atmosphere, i.e., with a smaller quantity of oxygen than that corresponding to the stoichiometric quantity required to completely combust the oil supplied, while the second phase is effected under an oxidizing environment, i.e., with an oxygen quantity exceeding the stoichiometrically required amount for combusting the oil supplied. Thus, approximately 80% of the stoichiometric oxygen requirement is used during the first phase and approximately 120% during the second phase. The first phase is conveniently continued until the charge is heated to a temperature of 850°-950° C. and the second phase is conveniently continued until a temperature of 1150°-1300° C. has been reached.

#### EXAMPLE 2

1500 kg of roasted copper raw material and 450 kg of fayalite slag were charged to an inclined rotary converter which has been preheated to 1000° C. The composition of the roasted material was mainly as shown in the following table:

65  
0.59% : Sb  
35.2% : Cu  
20.9% : S

28.7% : Fe  
11.7% : SiO<sub>2</sub>  
The composition of the slag was:

5  
35% : Fe  
65% : SiO<sub>2</sub>

The charged material was smelted with heat produced by burning oil in an oil oxygen-gas burner.

Heat was applied to the charged material for 24 minutes with a reducing flame, i.e., the amount of oxygen supplied was less than that corresponding to the stoichiometric requirement. The ratio of oil, in litres, to oxygen gas, in normal cubic meters, was 3:4.8. The temperature in the inclined rotary converter was raised to 900° C. Heat was then applied with an oxidizing flame for 26 minutes, i.e., the amount of oxygen supplied was greater than that corresponding to the stoichiometric requirement. The ratio of oil, in liters, to oxygen, in normal cubic meters, was 3:7.5. In this way the temperature of the smelt was raised to approximately 1200° C. The antimony content of the matte was determined at 0.33% Sb and the copper content at 48.3%.

20  
25  
30  
35  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415<br

by burning sulphur contained in said raw material, so that a smelt comprising a matte having a desired copper content and a copper-containing slag is formed and maintained at a temperature of 1100°-1300° C.; treating the smelt obtained with at least one reductant selected from the group consisting of coke, coal, oil, natural gas, pyrite, chalcopyrite, pyrrhotite and additional amounts of said sulphidic copper raw material, so that the copper content in the slag is decreased; transferring the smelt batchwise to a holding furnace in which the matte and the slag are mutually separated; treating the slag in the holding furnace during its passage therethrough to further decrease the copper content in the slag to a predetermined level; tapping-off the matte separated in the holding furnace and transferring said matte to a converter; and finally tapping-off the slag thus reduced and separated.

2. A method according to claim 1, wherein the slag in the holding furnace is treated by charging sulphide concentrates to the holding furnace.

3. A method according to claim 1, wherein the reductant comprises additional amounts of sulphidic copper raw material, comprising discontinuing the supply of

oxygen when at least 75% of the copper raw material has been charged to the furnace.

4. A method according to claim 1, wherein the oxygen charged to the furnace during the smelting process has the form of a gas containing 30-50% oxygen.

5. A method according to claim 1, wherein the temperature of the holding furnace is maintained by electric resistance heating or by combusting fuel.

6. A method according to claim 1, wherein the reduction is effected in the inclined rotary converter in a manner such that the copper content of the slag phase is less than 2%.

7. A method according to claim 1, wherein the copper content of the slag in the holding furnace is reduced to less

15 8. A method according to claim 1, wherein the temperature is maintained at 1150°-1250° C.

9. A method according to claim 1, wherein the temperature of the holding furnace is maintained at 1080°-1250° C.

20 10. A method according to claim 1, wherein the reduction in the holding furnace is effected by supplying coke, or coal, or by means of a reducing flame.

\* \* \* \* \*

25

30

35

40

45

50

55

60

65